

Oct. 15, 1940.

P. D. GERBER

2,218,489

PIEZOELECTRIC CRYSTAL

Filed May 31, 1939

*Fig. 1.*



*Fig. 2.*



*Fig. 3.*



*Fig. 4.*



Inventor

Paul D. Gerber

By

*J. D. Huff*

Attorney

## UNITED STATES PATENT OFFICE

2,218,489

## PIEZOELECTRIC CRYSTAL

Paul D. Gerber, Woodlynne, N. J., assignor to  
Radio Corporation of America, a corporation of  
Delaware

Application May 31, 1939, Serial No. 276,866

5 Claims. (Cl. 171—327)

This invention relates to the art of examining quartz piezoelectric crystals and particularly to a method of determining (a) the location of an electrical or X-axis, (b) the location of the positive and negative terminals of the said X-axis, and (c) whether the quartz is of the "right-handed" or "left-handed" variety.

Perfect quartz crystals, or "rock crystals" as they are sometimes called, occur in nature in the form of hexagonal bi-pyramids. Where any of the side or apex faces of the mother crystal remain intact, the location of an X-axis is a very simple matter since any line drawn parallel to that face in a plane normal to the Z axis coincides with an X-axis.

In the case of so-called "river-bed quartz," where the action of water over very long periods of time has worn away all of the natural faces of the quartz, and in the case of mere fragments of quartz, the location of the X-axes has heretofore been a most complicated procedure requiring the use of X-rays or other special electrical equipment.

Accordingly, the principal object of the invention is to provide an extremely simple and accurate method of determining the location of an X-axis in "river bed" and other imperfect quartz bodies.

In the production of X-cut (Curie cut) and Y-cut (Tillyer cut) crystal elements wherein the thickness dimension of the finished element is parallel to one or the other of the said axes, and its electrode faces are parallel to the optical (Z) axis, it is a matter of no moment to the person cutting the element whether the mother crystal is of the left-handed or right-handed variety, and he may be entirely oblivious as to which is the positive and which is the negative end of the axis which he has selected as a reference axis. However, in the case of more recently developed crystal cuts wherein the electrode faces of the element are tilted with respect to the optical (Z) axis, it is important (in the absence of a side or of an apex face which may be used as a reference plane) that the person cutting the mother crystal know whether the quartz upon which he is working is of the right-handed or left-handed variety, since the sense of direction of the angle of tilt required to achieve a desired characteristic (say, a "low temperature coefficient of frequency") may be, and usually is, different in the two types of quartz.

Accordingly, another and important object of the invention is to provide a method of locating 55 an X-axis in a quartz crystal and one which in

its practice likewise discloses the electrical sense or polarity of the said axis and also the type of quartz under inspection.

Other objects and advantages will be apparent and the invention itself will be best understood by reference to the following specification and to the accompanying drawing wherein

Figure 1 is a top plan view and Figure 2 is a side elevational view of one form of apparatus which may be employed in carrying out the 10 method of the invention,

Figures 3 and 4 are plan views of quartz slabs whose faces lie in planes normal to the optic axis, and wherein the said faces have been inspected and marked with reference characters 15 and lines as an aid in explaining the principle of the invention.

In carrying the invention into effect, it is first necessary to determine the location of the optical or Z-axis in the mother crystal. This may be 20 accomplished by any of the known methods or means. By way of example, the mother crystal, if it is transparent, or, alternatively, a transparent piece cut from any part of the mother crystal, may be immersed in cedar oil or equivalent substance and examined by means of polarized light while rotating the specimen until the colored light patterns or rings which are characteristic of the Z-axis are observed. The Z-axis at that time lies along the line of sight of the observer. The location of the Z-axis having been determined, a slab of any desired thickness is cut from the mother crystal in such a manner that the major faces of the slab lie in parallel planes which are substantially normal to the Z-axis.

In accordance with the invention, this slab is then etched as by immersing it overnight in a bath of hydrofluoric acid. When a 48 percent concentration of hydrofluoric acid is employed, an etching time of from, say, ten, to say, sixteen, hours is recommended. Irrespective of the exact duration of the etching time, it is desirable that both faces of the slab be equally subject to the action of the acid. Accordingly, the slab is preferably mounted on its edge in the bath so that both of its said faces are freely exposed to the acid. After being removed from its acid bath, rinsed and dried, the slab is ready for inspection.

Figs. 1 and 2 show an apparatus which may be employed in the inspection and marking of the blank. This apparatus is claimed per se in co-pending divisional application Serial No. 348,908, filed July 31, 1940, to the same inventor. In these figures, 1 designates a turntable upon which the quartz crystal slab Q is laid or clamped with one 55

of its etched plane faces A exposed. This turntable 1 is preferably arranged to accommodate slabs of various sizes and thicknesses. To this end, it is mounted for slideable movement on a 5 suitable base 2 and is adjustable in the vertical direction as by means of screw 3. An upright bracket 4 on the base 2 supports a ruler which may conveniently be in the form of a hinged plate 5 having a slot 6 therein for guiding a pencil 10 or stylus (not shown) over the exposed face of the crystal Q when the plate 5 is brought adjacent thereto.

A projector 7 containing a lamp (not shown) and a collimating lens 8 is directed towards the 15 crystal Q so that the parallel rays of light impinge the exposed face A of the slab at an angle of substantially 30°. A paralleloscope or collimator 9, which may consist simply of a  $\frac{1}{2}$  inch tube 15 to 20 inches long and having its inner 20 surface blackened, is provided for picking up light reflected in the return direction from the crystal. This collimator 9 is directed toward the upper face of the crystal at an angle of substantially 10° to 15°. The projector 7 and the collimator 9 are preferably adjustably supported 25 upon a common supporting rod 11 and must, in any event, extend in the same relative direction toward the crystal. The projector, the collimator, and the eye of the observer must, for optimum 30 accuracy, all reside in the same vertical plane, i. e., the plane containing the parallel rays of light which leave the collimating lens 8 and are reflected back into the collimator 9.

As a result of the etching process, the surfaces 35 (A and B) of the quartz which are normal to the optical or Z-axis reveal innumerable triangular crystalline pyramids of microscopic size. The planes of these crystalline particles are so arranged that only when the electrically negative 40 (-) end of an X-axis is pointed in the general direction of the source of light will the collimator pick up a sharply defined reflection of the light. Accordingly, the turntable 1 is rotated until such reflection is obtained, the final adjustment of the turntable being such that the reflected rays as viewed through the collimator 9 are of maximum intensity. The hinged plate or ruler 5 is then brought adjacent the upper face 45 A of the quartz slab Q and this reflection line or axis, a—a, Figs. 3 and 4, is preferably marked thereon as by inserting the point of the pencil or stylus in the straight slot 6 and drawing it therealong.

The reflection-axis a—a now marked on one 50 (A) of the two (A—B) parallel faces of the slab Q does not coincide with an X-axis but usually forms an angle of about 13° with an X-axis. This angle will vary from about 10° to 16° with the depth of the etching, and possibly with other 55 factors, such, for example, as the quality of the quartz and with minor inaccuracies in the orientation of the opposite faces A and B of the slab. This variation, however, is of substantially no moment as far as the practice of this invention is concerned.

In order to determine the substantially exact 60 location of an X-axis, the slab is turned over so that the corresponding area of its opposite face (B) is now presented to the parallel rays 65 of light from the projector 7, and the same steps of inspecting and marking the crystal are repeated. The reflection line noted in the inspection of the said opposite face (B) of the slab Q is shown by the broken line b—b in Fig. 3 and by the similarly designated solid line in Fig. 4. This

second reflection line b—b like the one a—a on the opposite face (A) of the slab Q does not coincide with an X-axis but, provided both faces have been equally exposed in the etching process and are otherwise similar, will be removed the same 5 number of degrees in the opposite direction from the X-axis. Thus, as the final step in locating the X-axis, it is merely necessary to bisect the opposite acute angles formed by the intersection of the reflection axes a—a, b—b. In both Figs. 10 3 and 4, the now located X-axis is designated by the dot-and-dash line X—X.

Since, as is well known to those skilled in the art, a crystal face which lies in a plane normal to the Z-axis exhibits three-fold symmetry, it 15 follows that the other two X-axes of the crystal may be located, if desired, by lines (not shown) which intersect the line X—X at angles of 120° in the same plane.

As previously set forth, it is only when the 20 electrically negative (-) end of an X-axis is pointed in the general direction of the source of light that the collimator 9 will pick up a sharply defined reflection of the light. Accordingly, when the polarity of the X-axis is of interest, 25 one or both of the surfaces A, B of the slab Q may be marked adjacent the opposite terminals of the X-axis with suitable indicia, say, the symbols — and +.

In order to determine the type of quartz (i. e., 30 whether it is "right-handed" or "left-handed" quartz), it is merely necessary to determine the direction in which the bisector or X-axis, X—X, need be rotated to coincide with the adjacent reflection axis a—a, or b—b. Thus, referring to 35 Fig. 3, wherein the plane A, which is marked with the reflection axis a—a, faces the observer, it will be noted that if the X-axis is to be rotated the shortest distance necessary to cause it to coincide with the said reflection axis a—a, it will have 40 to be rotated in a counter-clockwise direction. This is an infallible indication that the quartz specimen is of the "left-handed" variety. Conversely, as indicated in Fig. 4, if the X-axis must be rotated in a clockwise direction to cause it to 45 coincide with the adjacent reflection axis b—b, the quartz is of the right-handed variety.

The location of the Z and X-axes, the polarity of the X-axis, and the type of quartz all having been determined, the technician may proceed to 50 cut a crystal element from either the left-handed or right-handed slabs Q—Q', respectively, having any desired orientation with respect to these axes in the same manner that he would if these slabs had been cut from a perfect mother crystal.

Throughout this specification, the terms "right-handed" and "left-handed," as employed in designating the different varieties of quartz, are used in the sense now almost universally accepted in the art of piezoelectricity. That is to 55 say, the Herschel convention is employed. In agreement with this convention, a quartz crystal is designated as "right-handed" if it rotates the plane of polarization of plane polarized light traveling along the optical or Z-axis in a right-hand or clockwise direction, as viewed by an observer looking into the crystal from a point adjacent the source of light, and is designated "left-handed" if it rotates the plane of polarization to the left or in the counter-clockwise direction, as 70 viewed from the same point.

Also, the terms "positive" and "negative" as employed in designating the polarity of the opposite terminals of the X-axis are used in their ordinary and generally accepted electrical sense. 75

Various modifications of the invention will suggest themselves to those skilled in the art. Accordingly, the foregoing is to be interpreted as illustrative and not in a limiting sense except as required by the prior art and by the spirit of the appended claims.

5 What is claimed is:

1. Method of locating an electrical (X) axis of a crystal which comprises cutting a slab having a pair of substantially parallel faces at substantially right-angles to the optical (Z) axis of the crystal, etching said slab directing light upon one of the said etched parallel faces of said slab, marking the line of maximum reflection of the 10 light from said face, directing light upon the opposite etched face of said slab and marking its line of maximum reflection, and then bisecting the opposite acute angles formed by the intersection of said lines of maximum reflection.
2. Method of locating an electrical (X) axis of a crystal which comprises cutting a slab having a pair of substantially parallel faces at substantially right angles to the optical (Z) axis of the crystal, subjecting the said parallel faces 15 of said slab equally to the etching action of hydrofluoric acid for a prolonged period, projecting parallel rays of light upon one of the etched parallel faces of said slab while rotating said slab in its plane with respect to the source 20 of said light until said light is reflected from said face in the return direction, marking the line of maximum reflection of said light upon said face, projecting parallel rays of light upon the corresponding area of the opposite of the etched 25 faces of said slab while rotating said slab in its plane with respect to the source of said light until said light is reflected from the corresponding area of the said opposite face in the return 30 direction with maximum intensity, and then bisecting the opposite acute angles formed by the intersection of said lines of maximum reflection 35 and designating the bisector as an X-axis.

3. The invention as set forth in claim 2 where-  
in the said parallel rays of light impinge the re-  
spective etched faces of said slab at an angle of  
substantially 30° and the reflected of said par-  
allel rays are observed in the plane of the source 5  
of said light on an angle of from substantially  
10° to substantially 15°.

4. The invention as set forth in claim 2 and  
including the additional steps of determining in  
which direction the said bisector or X-axis must 10  
be rotated to coincide with the reflection line  
which is nearer the observer, and then utilizing  
the said slab as if it were of right-handed or  
left-handed crystalline structure as determined  
by whether it is necessary to rotate said X-axis 15  
in the clockwise or in the counter-clockwise di-  
rection, respectively, to cause it to coincide with  
said reflection line.

5. Method of determining the location and  
polarity of an X-axis of a crystal, said method 20  
comprising cutting a slab having substantially  
parallel faces at substantially right angles to  
the optical (Z) axis of the crystal, etching said  
slab directing light upon one of the etched par-  
allel faces of said slab, marking the line of 25  
maximum reflection of the light from said face  
and designating the immediate area adjacent  
that terminal of the said reflection line which  
is nearer the source of light as a negative (—)  
area and the immediate area adjacent the oppo- 30  
site terminal of said reflection line as a positive  
(+) area of said slab, repeating the said steps  
upon the corresponding area of the opposite  
etched parallel face of said slab, then bisecting  
the opposite acute angles formed by the inter- 35  
section of said reflection lines and finally des-  
ignating the bisector as an X-axis whose oppo-  
site terminals are of the polarity indicated at  
the adjacent corresponding terminal area of said  
reflection lines.

40 PAUL D. GERBER.